

Patented Feb. 26, 1929.

1,703,415

# UNITED STATES PATENT OFFICE.

HAMILTON BRADSHAW, OF WILMINGTON, DELAWARE; EDGAR H. NOLLAU, OF NEWBURGH, NEW YORK; AND RICHARD G. WOODBRIDGE, OF WILMINGTON, DELAWARE, ASSIGNORS TO E. I. DU PONT DE NEMOURS & COMPANY, OF WILMINGTON, DELAWARE, A CORPORATION OF DELAWARE.

## NITROCELLULOSE COMPOSITION.

No Drawing. Application filed December 21, 1921, Serial No. 523,991. Renewed March 21, 1924.

This invention relates to compositions containing, as an essential constituent, nitrocellulose which has a nitrogen content of more than 12.4% and which, in conjunction with suitable modifiers such as softeners, yields films having such properties as to render them technically valuable in the form of coatings for fabrics and other articles. More particularly our invention comprises nitrocellulose 5 solutions and plastics containing pyro nitrocellulose whose properties have been changed by a special treatment hereinafter described.

One object of our invention is to utilize pyro nitrocellulose in the manufacture of artificial leather of the coated fabric type, in coating compositions intended for the coating of paper, fabrics, and split leathers, and in general for leather substitute uses.

Another object of our invention is to utilize pyro nitrocellulose in the manufacture 20 of solutions such as lacquers, bronzing liquids, etc. for the coating of metal, wood, and other surfaces.

By pyro nitrocellulose is meant that grade 25 of nitrocellulose soluble in a mixture of 2 parts by volume of ether to one part of ethyl alcohol and having a nitrogen content of about 12.60%. A specific example of this grade of nitrocellulose is a product having a 30 solubility in ether-alcohol mixture of above 95%, generally above 99%, and a nitrogen content of 12.50 to 12.70%; such a product is commonly known as pyro and is hereinafter referred to as such.

Large quantities of pyro nitrocellulose remained unused after the cessation of the 35 World War. Attempts to use the pyro in "dope" solutions intended for the coating of fabrics showed that it differed from the regular type of pyroxylin used by the pyroxylin industry not only in having a higher nitrogen content but in possessing high viscosity, inferior solubility in the customary solvents, inferior affinity for castor, and other vegetable oils, and in general poorer qualities for film making purposes. Of the inferior qualities, those of high viscosity and low solubility in methyl and ethyl alcohol are not difficult to recognize even by those less skilled in the 40 art. The reduction in the viscosity of the pyro by boiling in water did not give to the resulting boiled material the desired qualities for use for coating purposes. For exam-

ple, artificial leather made from pyro previously boiled to reduce its viscosity appeared 55 visually to be satisfactory and might have been accepted as such by one not skilled in the art. However, the pyro-castor oil film exhibited a tendency to softness which peculiar 60 weakness grew more and more pronounced when the artificial leather was stored at atmospheric or higher temperature, the film becoming soft and mushy.

Worden's Technology of Cellulose Esters, 65 vol. 1, part 3, page 1691 states—"From 11.5%—12% N, are included the class of pyroxyllins—loosely defined and with no clear-cut lines of analytical demarcation, but including the nitrocellulose employed in artificial leather, lacquers, waterproofing solution, bronzing liquids, nitro-artificial filaments and the enameling and coating of hides and splits. The pyroxyllins are produced in an endless number of 'grades' for specific 70 purposes, where the solubility, 'flow,' adhesion, ability to mix with oils, tensile strength 75 and other factors are modified and manipulated in the process of nitration without at the same time varying but little the nitrogen content of the finished product." 80

The above statements by Worden are rather confirmatory of our results and indicate that the desirable limits of nitrogen content for pyroxylin for use in the artificial leather industry and for coating purposes in general 85 have by experience been found to be much lower than the nitrogen content of that grade of nitrocellulose designated as pyro.

We have discovered that by subjecting the pyro to a precolloiding treatment, in the 90 presence of diphenylamine, with a solvent mixture composed, for example, of approximately 2 parts ether by volume to 1 part denatured ethyl alcohol followed by a seasoning treatment at a temperature of, say, between 95 55 and 65°C. for about 15 to 25 days, that it gives coated products possessing superior qualities to those given by the pyro without previous precolloiding with ether-alcohol mixture and subsequent seasoning. We 100 have further found that this superior quality for coating purposes still persists and is even enhanced when the colloided pyro is still further seasoned at atmospheric temperature for many months.

The precolloiding and seasoning treatment 105

to which we may subject the pyro before using it for coating purposes may differ considerably in detail but we prefer to use a treatment substantially as follows:

5 We first dehydrate the pyro containing about 35% of water by forming it into blocks containing about 40 pounds dry weight. This we do by means of an hydraulic press. We then pump about 50 pounds of denatured 10 ethyl alcohol (formula containing  $\frac{1}{2}$  gallon benzene per 100 gallons of alcohol) through the pyro, thus displacing the water. We remove the excess of alcohol by squeezing the block of material under high pressure until 15 it weighs about  $53\frac{1}{3}$  pounds and contains about  $13\frac{1}{3}$  pounds alcohol and 40 pounds pyro (dry weight). After breaking up the block of alcoholized pyro by mechanical means, we place same in a mixer provided 20 with brine refrigeration and colloid it in the presence of about 0.5% of diphenylamine based on the dry weight of the pyro by the addition of about  $26\frac{2}{3}$  pounds of ether, in which the diphenylamine is previously dissolved, for each block of dehydrated pyro of the weight given above. After mixing for not more than one hour for the purpose of 25 thoroughly colloiding the pyro and thoroughly distributing the diphenylamine throughout the colloided mass, we reduce the colloid to a form convenient for subsequent handling by shaping it into blocks, then, by means of an hydraulic press, extruding the colloid through suitable perforations, and finally 30 granulating the extruded material on a cutting machine into grains of suitable size. These grains may, for example, be small cylinders about 0.4 of an inch long and about 0.2 of an inch in diameter, preferably provided 35 with about 7 evenly spaced, longitudinal perforations each about 0.02 of an inch in diameter for facilitating escape and recovery of solvent.

The bulk of ether-alcohol solvent may be removed from the grains of seasoning, if desired, in a suitable solvent recovery apparatus at a temperature of about  $60^{\circ}$  C., the solvent which vaporizes being condensed. The colloided grains, which have been thus 40 treated to recover the solvent, are then further seasoned by heating in hot water for about 15 to 25 days at a temperature of about  $60^{\circ}$  C., after which the colloided grains are air dried at a temperature of about  $60^{\circ}$  C. 45 until the moisture in the colloid is reduced to about 1.0 to 2.0%. The colloided grains are then stored in air-tight receptacles for a still further seasoning treatment at atmospheric temperature, which treatment may extend 50 over a period of many months, (usually more than 4 months), until the viscosity of a standard testing solution of the colloided grains is reduced to 200 seconds or below when measured by the procedure hereinafter described.

55 We have found that the pyro precolloided

and seasoned as above described does not give coatings, i. e., films, with the tendency to soften and become mushy on storage which is characteristic of pyro which has been boiled to reduce its viscosity, but instead gives 70 coatings of satisfactory toughness which retain this quality during storage for a considerable period of time. In fact experiments show that the degree of deterioration of the new coatings or films upon ageing, due to the 75 gradual and inevitable degradation of the nitrocellulose, is even less than the deterioration which occurs in coatings made according to the present day standard methods from nitrocellulose having less than 12% nitrogen. 80

The improved quality for coating purposes of the pyro which has been precolloided and seasoned substantially as above described, is to be attributed to a number of factors. Of these, the most readily measured is the very 85 gradual change in the viscosity characteristic which occurs during the seasoning process, which we believe tends to bring the viscosity characteristics of all component parts of the colloid to the same point. For example, a standard testing solution of a sample of pyro before precolloiding gave a viscosity of 850 seconds at  $28^{\circ}$  C. by the so-called steel ball method, the time being that required for a 90  $\frac{1}{4}$ " steel ball to fall in a 1.25" tube through 10" of the standard testing solution, which solution is made by dissolving 16 ounces of the pyro in a gallon of solvent mixture composed of benzene 50 parts, denatured ethyl alcohol 25 parts, and ethyl acetate 25 parts. After precolloiding with ether-alcohol mixture and seasoning for about 20 days at a temperature of  $60^{\circ}$  C., 4 days of which were in solvent recovery apparatus for the purpose of recovering the ether and alcohol, and 15 95 days of which were in hot water at  $60^{\circ}$  C., the remaining day being in air, the viscosity of the colloid was reduced to about 400 seconds. Further seasoning of the colloid for 100 35 months at atmospheric temperature gradually reduced the viscosity of the colloid to about 85 seconds. A seasoning treatment at atmospheric temperature for about 20 months will ordinarily effect a satisfactory reduction 105 in viscosity.

An important feature of our invention is that the diphenylamine present in the pyro colloid decidedly retards the development of rancidity of the castor oil or other vegetable oils used as softeners in the manufacture of artificial leather of the nitrocellulose coated fabric type. This is a very important advantage in the manufacture of artificial leather. We do not limit ourselves to the amount of diphenylamine which we may have present in the precolloiding of the pyro, but have found that up to 1.0% of diphenylamine has no objectionable influence on the seasoning of the pyro colloid, and an increased amount, for example up to about 4%, is an 110 115 120 125 130

advantage in retarding the development of rancidity.

To prepare compositions suitable for coating fabrics we mix with the precolloided pyro 5 a softener which may be either a non-solvent softener such as a non-drying vegetable oil (e. g. castor oil) or a solvent softener such as dibutyl phthalate, or preferably both. These compositions are of course applied to 10 the fabric in the form of their solutions, the volatile solvent consisting usually of an active solvent and a diluent.

Typical coatings or films made from the precolloided pyro may have, for example, the 15 following compositions:

|                        | Parts<br>by weight. | Per cent.    |
|------------------------|---------------------|--------------|
| I. Precolloided pyro   | 1.00                | 30.8 - 28.70 |
| Castor oil             | 1.63-2.13           | 50.0 - 56.65 |
| Pigment                | 0.625               | 19.2 - 16.65 |
| II. Precolloided pyro  | 1                   | 23.55-21.05  |
| Blown rapeseed oil     | 2.65-3.13           | 61.75-65.80  |
| Pigment                | 0.625               | 14.70-13.15  |
| III. Precolloided pyro | 1                   | 33.3         |
| Castor oil             | 1.25-1.1            | 41.6 - 36.65 |
| Dibutyl phthalate      | 0.13-0.28           | 4.3 - 9.05   |
| Pigment                | 0.62-0.62           | 21.15        |

The above compositions represent the non-25 volatile portion of the solutions from which the coatings or films are produced.

As the volatile solvent there may be used for example a mixture of 50 parts benzene, 25 parts ethyl acetate, and 25 parts denatured 30 alcohol. From 7 to 8 parts of this solvent mixture may be used to 1 part of the non-volatile composition of any of the above examples to form the coating solution. The pigment must of course be ground in a portion, or if necessary all, of the oil before it 35 can be satisfactorily incorporated into the nitrocellulose solution.

Many solvent mixtures other than the one described above may of course be used. For 40 example as the active solvent there may be used either acetone, acetone oils, methyl acetone (a commercial mixture containing methyl acetate, methyl alcohol, and acetone), or an ether-alcohol mixture; and as the diluent there may be used, for example, ethyl alcohol, benzine or benzol.

It will of course be understood that various 45 modifications, not specifically described above, may be made in our new process and 50 product without departing from our invention.

We claim:

1. A coating composition consisting essentially of precolloided and seasoned pyro nitrocellulose and a softener therefor.
2. A coating composition consisting essentially of precolloided and seasoned pyro nitrocellulose and a softener therefor comprising a non-drying vegetable oil.
3. A coating composition consisting essen-

tially of precolloided and seasoned pyro nitrocellulose and a softener therefor comprising a non-drying vegetable oil and a solvent softener.

4. A coating composition comprising nitrocellulose of from 12.5 to 12.7% nitrogen content, diphenylamine, a vegetable oil, and dibutyl phthalate. 65

5. The process of making a coating composition which comprises colloiding a nitrocellulose of more than 12.4% nitrogen content, comminuting the resulting colloid, seasoning the comminuted mass for from about 2 to 4 weeks at a temperature of about 60° C., further seasoning the mass at about atmospheric temperature until a standard testing solution made therefrom shows a viscosity of less than 200 seconds when measured by the method hereinbefore described, and then dissolving the seasoned comminuted mass in a 70 nitrocellulose solvent. 75

6. The process of making a coating composition which comprises dissolving in a nitrocellulose solvent a nitrocellulose mass obtainable by colloiding a nitrocellulose of 80 more than 12.4 nitrogen content, comminuting the resulting colloid, seasoning the comminuted mass for from about 2 to 4 weeks at a temperature of about 60° C., further seasoning the mass at about atmospheric temperature until a standard testing solution made therefrom shows a viscosity of less than 200 seconds when measured by the method hereinbefore described. 85

7. The process of making a coating composition which comprises colloiding a nitrocellulose of from about 12.4 to 12.7% nitrogen content, comminuting the resulting colloid, seasoning the comminuted mass partly at an elevated temperature, until a standard testing solution made therefrom shows a viscosity of less than 200 seconds when measured by the method hereinbefore described, and then dissolving the seasoned, comminuted mass in a nitrocellulose solvent. 90 95

8. A coating composition comprising a precolloided and seasoned nitrocellulose having a nitrogen content of from about 12.4 to 12.7%, a vegetable oil, and dibutyl phthalate. 100

9. A coating composition comprising a 110 precolloided and seasoned nitrocellulose having a nitrogen content of from about 12.4 to 12.7%, a non-solvent softener, and a neutral phthalate.

In testimony whereof we affix our signatures. 115

HAMILTON BRADSHAW.  
EDGAR H. NOLLAU.  
RICHARD G. WOODBRIDGE.